

1

3,676,147

**METHOD OF SPECTRALLY SENSITIZING PHOTOGRAPHIC SILVER HALIDE EMULSIONS**

Simone J. Boyer and Roger Caridi, Vincennes, France, assignors to Eastman Kodak Company, Rochester, N.Y.  
No Drawing. Filed Nov. 28, 1969, Ser. No. 880,944  
Claims priority, application France, Dec. 24, 1968,

180,194

Int. Cl. G03c 1/16, 1/18, 1/20

U.S. Cl. 96—130

13 Claims

**ABSTRACT OF THE DISCLOSURE**

Light sensitive silver halide is spectrally sensitized by dispersing a substantially water-insoluble photographic spectral sensitizing dye into a water-soluble organic liquid without dissolving the dye, and incorporating the dispersion into a liquid photographic silver halide emulsion. Novel dispersions of dyes are also provided.

This invention relates to novel photographic processes and more particularly to novel processes for spectrally sensitizing photographic silver halide emulsions. It also relates to novel photographic materials and processes.

The conventional method of sensitizing light sensitive silver halide consists of dissolving the sensitizing dye in an appropriate organic solvent, such as methyl alcohol, ethyl alcohol, acetone, etc., and adding the resulting solution to a liquid photographic silver halide emulsion. While this general method has provided a commercially feasible means for incorporating sensitizing dyes into silver halide emulsions, it still requires considerable care and extra manipulative steps in adjusting the volume of solvent to quantities that are compatible with the particular emulsion and still produce the desired results. Also, it is well known that excessive solvent engenders disadvantageous diffusion or wandering of the sensitizing dyes in the emulsions.

It is, accordingly, an object of this invention to provide a new method for spectrally sensitizing light sensitive silver halide.

Another object of this invention is to provide novel dispersions of spectral sensitizing dye.

Other objects of this invention will be apparent from this disclosure and the appended claims.

In accordance with one embodiment of this invention, a process is provided for spectrally sensitizing photographic silver halide which comprises: dispersing a substantially water-insoluble photographic spectral sensitizing dye into a water-soluble organic liquid without dissolving the dye; and, incorporating the dispersion into a liquid photographic silver halide emulsion.

In accordance with another embodiment of this invention, novel dye dispersions are provided which comprise undissolved particles of a photographic spectral sensitizing dye in a water-soluble organic liquid.

In still another embodiment of this invention, novel compositions are provided which comprise a hydrophilic colloid containing undissolved particles of photographic spectral sensitizing dye in a water-soluble organic liquid in which said dye is substantially insoluble. Such composition can be either liquid or solid; either form is useful for spectrally sensitizing liquid photographic silver halide emulsions.

The dye dispersions of the invention are especially useful in coating processes which require low amounts of organic solvent. The dye dispersions are stable and can be conveniently stored or transported.

The compositions of dye in organic liquid can be prepared in any convenient manner. Ball milling the dye and organic liquid gives highly satisfactory results. Ad-

2

vantageously, the liquid contains dye particles which have an average diameter of up to about 1.0 micron.

Organic liquids which can be used in the practice of this invention are water-soluble materials, and are liquids below about 30° C. Organic liquids can be used which are not solvents for the photographic sensitizing dye that is being used. Such organic liquids are oily materials. They should not have any adverse effects on the photographic emulsion in which they are incorporated. Also useful are organic liquids which are solvents for the dye. Such organic liquids, e.g., methanol, ethanol or isopropanol are used at sufficiently low levels, compared to the quantity of dye, that only very small amounts of dye are dissolved. Both types of liquids function to separate, or prevent agglomeration of the dye particles. Such separation is essential to effective spectral sensitization.

Typical organic liquids that are not dye solvents which can be used in the invention are represented by the following formula:



25 wherein R represents a hydrogen atom or a lower alkyl group containing 1 to 4 carbon atoms, e.g., methyl, ethyl, butyl, etc.; R<sub>1</sub> represents a hydrogen atom or a methyl group; R<sub>2</sub> represents a hydrogen atom, an alkyl group containing from 1 to 3 carbon atoms, e.g., methyl, ethyl, propyl or isopropyl, a hydroxymethyl group or an acetoxy-methyl group; and R<sub>3</sub> represents a divalent alkylene group containing from 1 to 4 carbon atoms, e.g., —CH<sub>2</sub>—, —CH(CH<sub>3</sub>)—, —(CH<sub>2</sub>)<sub>2</sub>—, —(CH<sub>2</sub>)<sub>3</sub>— or



35 and wherein the sum of the carbon atoms in said R<sub>1</sub>, R<sub>2</sub> and R<sub>3</sub> is a positive integer of from 1 to 4. Typical useful liquids embraced by Formula I above include glycerol, monoacetin, ethylene glycol, methylglycol, (monomethyl ether of ethylene glycol), ethyl glycol ether, propyl glycol ether, butyl glycol ether, 1,3-propylene glycol, 1,3-butylene glycol, 1,4-butylene glycol, 2,3-butylene glycol, isobutylene glycol (2-methyl-1,2-propanediol), 2-methyl-2,3-butanediol, 3-methyl-1,3-butanediol, 1,2-pentanediol, 1,4-pentanediol, 2,3-pentanediol, 1,5-pentanediol, etc. Glycerol and methylglycol are the preferred solvents herein.

Also useful in the practice of this invention are organic liquids which are solvents for spectral sensitizing dyes. Such liquids are used in sufficiently small amounts, relative to the quantity of spectral sensitizing dye, that no substantial amounts of dye are dissolved. Preferably, such liquids have a dissolving power for the dyes of less than 10 grams of dye per liter of solvent at 20° C. Useful organic liquids of this class include alcohols having from 1 to 4 carbon atoms, such as methanol, ethanol, n-propanol, iso-propanol, n-butanol, iso-butanol or tert-butanol; acetone; and, dimethylformamide. Such solvents provide less tacky dye dispersions than similar dispersions made with relatively high boiling organic liquids.

60 Especially good results are obtained with a mixture of one or more organic liquids which are non-solvents for the dye, together with one or more organic liquids which are solvents for the dye. A typical useful solvent mixture of this type is a mixture of methanol (which is a solvent for most sensitizing dyes) together with glycerol (which is a non-solvent for most sensitizing dyes). Particularly good results are obtained with an organic liquid mixture comprising about 80 to 95 parts by weight solvent (e.g., methanol) and 20 to 5 parts by weight of a non-solvent liquid (e.g., glycerol) and preferably about 90 parts by weight solvent and 10 parts by weight non-solvent.

The spectral sensitizing dye is dispersed in the organic

liquid without dissolving the dye. As used herein, the term "without dissolving the dye" means that no substantial amount of dye is dissolved. Preferably, less than about 5% by weight of the total dye mixed with the liquid is dissolved. Essentially no dye is dissolved when the dye is insoluble in the organic liquid. When the organic liquid is one which will dissolve the dye, the solvent is used in such small concentrations relative to the total amount of dye that no substantial amount of dye is dissolved. Typical solutions of sensitizing dye in organic solvent, e.g., methanol, contain about 1 to 3 grams dye per liter of solvent. In accordance with this invention, preferably about 5 to 20 cc. of solvent are used per gram of dye.

This invention can be practiced with any of the photographic spectral sensitizing dyes. The invention is especially useful with the dyes that are substantially insoluble in aqueous solutions, e.g., dyes which have a solubility in water (at 20° C.) of less than about 1%. Typical dyes which can be used in the practice of this invention are described in the following patents, the disclosure of which are incorporated herein by reference.

Zeh et al. U.S. Pat. No. 2,068,047, issued 1/19/37  
 Brooker U.S. Pat. No. 2,078,233, issued 4/27/37  
 Koslowsky U.S. Pat. No. 2,107,379, issued 2/8/38  
 Mees U.S. Pat. No. 2,158,883, issued 5/16/39  
 Brooker et al. U.S. Pat. No. 2,161,331, issued 6/6/39  
 Brooker U.S. Pat. No. 2,170,807, issued 8/29/39  
 Brooker U.S. Pat. No. 2,177,402, issued 10/24/39  
 Brooker U.S. Pat. No. 2,177,403, issued 10/24/39  
 Carroll et al. U.S. Pat. No. 2,177,635, issued 10/31/39  
 Carroll U.S. Pat. No. 2,206,076, issued 7/2/40  
 Brooker U.S. Pat. No. 2,211,762, issued 8/20/40  
 Brooker et al. U.S. Pat. No. 2,213,238, issued 9/3/40  
 Brooker U.S. Pat. No. 2,307,916, issued 1/12/43  
 Brooker et al. U.S. Pat. No. 2,313,922, issued 3/16/43  
 Schneider U.S. Pat. No. 2,374,505, issued 4/24/43  
 Falleson et al. U.S. Pat. No. 2,378,917, issued 6/26/45  
 Brooker U.S. Pat. No. 2,454,629, issued 11/23/48  
 Thompson U.S. Pat. No. 2,535,993, issued 12/26/50  
 Carroll et al. U.S. Pat. No. 2,950,196, issued 8/23/60  
 Brooker et al. U.S. Pat. No. 2,955,939, issued 10/11/60  
 Jones U.S. Pat. No. 2,961,318, issued 11/22/60  
 Brooker et al. U.S. Pat. No. 2,194,805, issued 7/13/65  
 Tabor et al. U.S. Pat. No. 3,335,010, issued 8/8/67  
 Brooker et al. U.S. Reissue No. 24,292, reissued 3/19/57  
 I.G., British Pat. No. 434,235, accepted 8/28/35

The following table lists a number of cyanine dyes that are used in the examples hereinafter to illustrate the invention.

TABLE 1

| Dye No.:   | Compound                                                                                            |
|------------|-----------------------------------------------------------------------------------------------------|
| I -----    | 1'-ethyl-2-methylthia-4'-cyanine iodide                                                             |
| II -----   | 3,3'-diethyl-9-methylselenacarbocyanine bromide                                                     |
| III -----  | 1,1'-diethyl-2,2'-cyanine iodide                                                                    |
| IV -----   | 3-ethyl-5-[ (3-ethyl-2(3H)-benzothiazolylidene)isopropylidene]-2-thio-2,4-oxazolidinedione          |
| V -----    | 9-ethyl-3,3'-di(β-methoxyethyl)-5,5'-diphenyloxacarbocyanine iodide                                 |
| VI -----   | Anhydro-5',6',6'-tetrachloro-1,1'-diethyl-3,3'-di(3-sulfobutyl)benzimidazolocarbocyanine hydroxide  |
| VII -----  | 5[(3-ethyl-2(3H)-naphtho[2,1]oxazolylidene)ethylene]-3-n-heptyl-1-phenyl-2-thiohydantoin            |
| VIII ----- | 5-(3-ethyl-2(3H)-benzoxazolylidene)-3-phenylrhodanine                                               |
| IX -----   | Anhydro-5,5'-dichloro-3,9-diethyl-3'-(3-sulfobutyl)thiacarbocyanine hydroxide                       |
| X -----    | 5-[di(3-ethyl-2(1H)-naphtho[1,2]thiazolylidene)isopropylene]-1,3-di-(β-methoxyethyl)barbituric acid |

TABLE I—Continued

| Dye No.:  | Compound                                                              |
|-----------|-----------------------------------------------------------------------|
| XI -----  | 3-ethyl-5-[1-(4-sulfobutyl)-4(1H)-pyridylidene]rhodanine, sodium salt |
| XII ----- | Anhydro-3-ethyl-9-methyl-3'-(3-sulfobutyl)thiacarbocyanine hydroxide  |

It will be understood that cyanine dye salts such as above Dye Nos. I, II, III and V include not only the specified iodide and bromide salts, but also the chloride, sulfamate, thiocyanate, perchlorate, p-toluenesulfonate, methyl sulfate, etc. salts. Also, Dye No. XI includes any of the alkali metal salts such as lithium, potassium, etc.

In preparing the novel dispersions of the invention, the weight proportions of the water-soluble liquid (which is a non-solvent for the dyes) to dye can vary over a wide range, such as from about 100:5 to 100:50, but preferably from about 100:10 to 100:40, respectively. Liquids which are dye solvents are advantageously used in weight proportions of about 5 to 20 parts solvent per each part by weight of dye.

Those dispersions of the invention containing a binder such as gelatin can vary widely in the proportions of dye to gelatin, but the best results for sensitizing purposes are obtained with compositions wherein the dye varies from 20 to 40%, based on the total weight of dye plus binder. For spectrally sensitizing photographic silver halide emulsions, the dispersions of the dyes can also contain two or more dyes in each dispersion or dispersions containing a single dye can also be used in combinations of two or more such dispersions. Generally, the concentration of dye incorporated into the emulsions by the method of the invention for optimum sensitivity varies depending on the dye and emulsion about from 0.20 to 4.0 grams of dye per mole of silver halide in the emulsion. The dye dispersions of the invention can be readily incorporated into the emulsions by any suitable method such as mixing, mechanical blending, etc.

Compositions of the invention consisting essentially of organic liquid and dye can be added directly to liquid photographic silver halide emulsions to obtain good spectral sensitization. If desired, the composition of the invention can be dispersed in a hydrophilic colloid. The dispersion of dye-organic liquid in hydrophilic colloid can be used in liquid or solid form to sensitize liquid silver halide emulsions. The hydrophilic colloid used with the dye-organic liquid can be any colloid which is compatible with the photographic emulsions, such as any of the hydrophilic colloids referred to below. Gelatin is especially useful. The colloid is preferably free from silver halide, or, the mixture comprises a substantial amount of dye which is unadsorbed on any silver halide present in the colloid.

This invention is useful in spectrally sensitizing any liquid photographic silver halide emulsion. The light sensitive silver halide can be dispersed in any hydrophilic colloid (binder) that is satisfactory for dispersing silver halides, for example, gelatin, albumin, agar-agar, gum arabic, alginic acid, polyvinyl alcohol, polyvinyl pyrrolidone, cellulose ethers, partially hydrolyzed cellulose acetate, and the like. The hydrophilic colloid can also contain dispersed polymerized vinyl compounds, such as those disclosed in U.S. Pats. 3,142,568; 3,193,386; 3,062,674 and 3,220,844 and include the water insoluble polymers of alkyl acrylates and methacrylates, acrylic acid, sulfoalkyl acrylates or methacrylates and the like.

While the examples herein are illustrated with silver bromoiodide emulsions, it will be apparent that other silver halide emulsions such as silver chloride, silver bromide, silver chlorobromide, silver chlorobromoiodide, etc. can also be efficiently sensitized in like manner with the novel dye dispersions of the invention.

The emulsions prepared in accordance with the invention may be coated on any suitable photographic support such as cellulose acetate, cellulose acetate butyrate, polyesters such as poly(ethylene terephthalate), polyethylene,

polypropylene, paper, glass, and the like, to produce spectrally sensitized photographic elements.

The photographic emulsions prepared in accordance with the novel method of this invention may contain such addenda as chemical sensitizers, e.g., sulfur sensitizers (e.g., allyl thiocarbamate, thiourea, allylisothiocyanate, cystine, etc.), various gold compounds (e.g., potassium chloroaurate, auric trichloride, etc. (see Baldsiefen, U.S. Pat. No. 2,540,085, issued Feb. 6, 1951; Damschroder, U.S. Pat. No. 2,597,856, issued May 27, 1952 and Yutzy et al. U.S. Pat. No. 2,597,915, issued May 27, 1952), various palladium compounds such as palladium chloride (Baldsiefen, U.S. Pat. No. 2,540,086, issued Feb. 6, 1951), potassium chloropalladate (Stauffer et al., U.S. Pat. No. 2,598,079, issued May 27, 1952), etc., or mixtures of such sensitizers, antifoggants such as ammonium chloroplatinate (Trivelli et al., U.S. Pat. No. 2,566,245, issued Aug. 28, 1951), ammonium chloroplatinite (Trivelli et al., U.S. Pat. No. 2,566,263, issued Aug. 28, 1951), benzotriazole, nitrobenzimidazole, 5-nitroimidazole, benzidine, mercaptans, etc. (see Mees—"The Theory of the Photographic Process," MacMillan Pub., 1942, page 460), or mixtures thereof. The silver halide emulsions of the invention can be hardened with any suitable hardener, including aldehyde hardeners such as formaldehyde, and mucochloric acid, aziridine hardeners, hardeners which are derivatives of dioxane, oxypolysaccharides such as oxy starch or oxy plant gums, and the like. The emulsion layers can also contain additional additives, particularly those known to be beneficial in photographic emulsions, including, for example, lubricating materials, stabilizers, speed increasing materials, absorbing dyes, plasticizers, and the like. These photographic emulsions can also contain in some cases additional spectral sensitizing dyes. Furthermore, these emulsions can contain color forming couplers or can be developed in solutions containing couplers or other color generating materials. Among the useful color formers are the monomeric and polymeric color formers, e.g., pyrazolone color formers, as well as phenolic, heterocyclic and open chain couplers having a reactive methylene group. The color forming couplers can be incorporated into the photographic silver halide emulsion using any suitable technique, e.g., techniques of the type shown in Jelley et al. U.S. Pat. 2,322,027, issued June 15, 1943, Fierke et al. U.S. Pat. 2,801,171, issued July 30, 1957, Fisher U.S. Pats. 1,055,155 and 1,102,028, issued Mar. 4, 1913 and June 30, 1914, respectively, and Wilmanns U.S. Pat. 2,186,849, issued Jan. 9, 1940. They can also be developed using incorporated developers such as polyhydroxybenzenes, aminophenols, 3 - pyrazolidones, and the like.

The following examples are included for a further understanding of this invention.

#### EXAMPLE 1

1.350 g. of Dye No. I are milled for 6 hours in a ball-mill with 6 cc. of methylglycol to give a dye dispersion wherein the dye particles have an average diameter less than about 1 micron. To this dispersion 18 g. of a 15% gelatin solution are then added. The mixture is homogenized in a ball-mill for 15 minutes. The mixture is then air dried, formed into flakes so as to be readily bottled and stored at room temperature in a brown glass bottle. A suitable sample of the mixture is used to determine the dye content of the mixture. In the present example, the dye concentration is 31.5% by weight.

#### EXAMPLES 2-11

The procedure described in above Example 1 is repeated with each of the other dyes listed in Table 1 above, namely, Dye Nos. II to XI to give the corresponding dye dispersions in the concentrations listed in the following table.

TABLE 2

| Dye No. | Conc. of—      |                            | Gelatin solution          |                             | Dye conc.<br>in final<br>mix (wt.<br>percent) |
|---------|----------------|----------------------------|---------------------------|-----------------------------|-----------------------------------------------|
|         | Dye<br>(grams) | Methyl-<br>glycol<br>(cc.) | Total<br>soln.<br>(grams) | Conc.<br>gelatin<br>(grams) |                                               |
| II      | 3              | 12                         | 36                        | 15                          | 35                                            |
| III     | 0.750          | 6                          | 18                        | 15                          | 21                                            |
| IV      | 3              | 12                         | 36                        | 15                          | 35                                            |
| V       | 3.45           | 14                         | 42                        | 15                          | 33                                            |
| VI      | 3.45           | 14                         | 42                        | 15                          | 23                                            |
| VII     | 2              | 8                          | 42                        | 10                          | 29                                            |
| VIII    | 3              | 10                         | 60                        | 10                          | 29.5                                          |
| IX      | 3.5            | 9.5                        | 62                        | 10                          | 35.8                                          |
| X       | 0.5            | 4                          | 12                        | 10                          | 30.5                                          |
| XI      | 0.4            | 5                          | 12                        | 10                          | 25.5                                          |

#### EXAMPLE 12

A negative gelatino silver bromoiodide emulsion is digested to optimum sensitivity with a labile sulfur compound and a soluble gold salt. It is then divided into two portions (a) and (b) and each portion is optically sensitized by adding the following mixture to the melted emulsion:

|             |       |
|-------------|-------|
| G.          |       |
| Dye No. I   | 0.450 |
| Dye No. II  | 1     |
| Dye No. III | 0.250 |

per 10 moles of silver halide in the emulsion. In portion (a), the dye mixture is added in solution in conventional solvents such as methanol. In portion (b), the dye mixture is milled with methyl glycol and dispersed in gelatin as described in above Example 1 and the resulting dispersion is then added to the emulsion.

Each of these two emulsions is kept at 40° C. for 20 minutes and then each is coated onto a separate cellulose acetate film support. The coated samples are sensitometrically tested by successive exposures of each sample to white light and through Wratten Filters No. 25 which transmits light at wavelengths longer than about 590 nm., No. 47 which transmits light in the region of about from 350 to 530 nm., and No. 58 which transmits light in the region of about from 470 to 615 nm., followed by development for about 6 minutes at room temperature in Kodak D-19 developer which has the following composition:

|                                |      |
|--------------------------------|------|
| G.                             |      |
| N-methyl-p-aminophenol sulfate | 2.0  |
| Sodium sulfite (anhydrous)     | 90.0 |
| Hydroquinone                   | 8.0  |
| Sodium carbonate (monohydrate) | 52.5 |
| Potassium bromide              | 5.0  |
| Water to make 1.0 liter.       |      |

then fixed, washed and dried. The resulting speed values for the emulsions sensitized by processes (a) and (b) are shown to be identical by the test procedure of this example. Similar good results of sensitization are likewise obtained when the dispersion of the dyes in methylglycol is used directly, without binder or drying, in the silver halide emulsion.

#### EXAMPLE 13

The photographic tests carried out in this example are similar to those described in above Example 12, except that the preparation of the milled dyes dispersed in gelatin were made 3 months before. The sensitometric results, which are identical with those described in the preceding example, show the good keeping properties of the dye dispersions of the invention.

#### EXAMPLE 14

A negative silver halide emulsion similar to that described in above Example 12 is optically sensitized with the dye mixture:

|            |      |
|------------|------|
| G.         |      |
| Dye No. IV | 1.00 |
| Dye No. V  | 1.13 |
| Dye No. VI | 1.13 |

per 10 moles of silver halide in the emulsion, in accordance with methods (a) and (b) described in Example 12. The tests show that the speeds of the emulsions optically sensitized by methods (a) and (b) in this example are identical to white light, to light transmitted through Wratten Filter No. 47 and to light transmitted through Wratten Filter No. 58.

#### EXAMPLE 15

A mixture of Dye Nos. I, II and III, in the proportions given in above Example 12, is milled with 10 cc. of methyl glycol until the dye particles have an average diameter less than about 1 micron. The resulting dye paste is dispersed in 12 g. of a 15% aqueous gelatin solution, dried and then used to sensitize a photographic silver halide emulsion, as described in Example 12. The sensitivity of this emulsion is substantially the same as that of the emulsion prepared in Example 12 by method (a), except that the speed loss in white light as compared to the control is 0.08 log E.

#### EXAMPLE 16

This example is identical with that of Example 15, except that the mixture of dyes is milled with 12 cc. of glycerol and taken up with 20 g. of a 10% aqueous gelatin solution. The sensitometric results of this example are identical with those of above Example 15.

#### EXAMPLE 17

The mixture of dyes described in Example 14 is milled with 10 cc. of methylglycol, taken up with 30 g. of 10% gelatin solution and dried. The dry mixture is used for optically sensitizing a photographic emulsion by the method described in Example 12.

The emulsion sensitized with the solid mixture (method b) shows a speed loss of 0.10 log E as compared to the control (method a), in white light.

#### EXAMPLE 18

This example and results thereof are identical with those of Example 17, except that the dye mixture is milled with 15 cc. of glycerin.

In Examples 15, 16, 17 and 18, the small loss in sensitivity appears to result from loss of dyes when the mixtures are recovered from the ball-mills.

#### EXAMPLE 19

500 mg. of Dye II are milled for 24 hours in a ball-mill in the presence of 5 cc. of methanol. Less than 5% by weight of the total amount of dye is dissolved in methanol. 50 cc. of a 10% aqueous gelatin solution are then added and the mixture is effected in the same ball-mill at 40° C. for 2 hours. This mixture is coated on unsubbed poly(ethylene terephthalate) support, in the form of a film having a thickness of 30 $\mu$  to 40 $\mu$ . After drying, the film which adheres to the support due to the effect of electrostatic charges is readily stripped from the base. It is broken into flakes by being passed through a grate under the action of compressed air. It is then readily weighed, titrated and stored. The mixture, which contains about 8% by weight of dye, is used to spectrally sensitize an emulsion as described in Example 12. The spectral sensitometric results obtained, as in Example 12, are identical with those obtained by conventional spectral sensitization methods (i.e., when the dye is dissolved in an aqueous solution of methanol and added to the emulsion).

#### EXAMPLE 20

The procedure of Example 19 is repeated except that the 5 cc. of methanol are replaced with 5 cc. of a 90:10 methanol-glycerin mixture. Identical sensitometric results are obtained.

#### EXAMPLES 21-26

The procedures of Examples 19 and 20 are repeated, except that in each Example Dye II is replaced with 500

mg. of Dyes I, III and XII. The sensitometric results, obtained as in Example 12, are identical to those obtained when the dyes are added to the same emulsion from methanol solutions.

5 It is well known in the photographic art that effective spectral sensitization of light sensitive silver halide depends on the dyes being adsorbed to the silver halide grains. See Mees and James, *The Theory of the Photographic Process*, 3d. edition, published by the MacMillan Company, 1966, page 236, column 2. One skilled in the photographic art would not expect particles of spectral sensitizing dyes, which are insoluble in aqueous systems, to migrate through a hydrophilic colloid and become efficiently adsorbed to the silver halide.

10 It will be apparent from all the foregoing that any other of the dyes mentioned in Table 1 above, as well as still other known cyanine sensitizing dyes that are water-insoluble, can be substituted in the procedures of the above examples to give generally similar useful results.

20 Also, any other of the mentioned water-soluble dihydroxy-alkanes or lower monoalkyl ether derivatives thereof which are non-solvents for the sensitizing dyes, glycerol, monoacetic, ethylene glycol, methylglycol, ethyl glycol ether, propyl glycol ether, butyl glycol ether, 1,3-propylene

25 glycol, 1,3-butylene glycol, 1,4-butylene glycol, 2,3-butylene glycol, isobutylene glycol, 2-methyl-2,3-butanediol, 3-methyl-1,3-butanediol, 1,2-pentanediol, 1,4-pentanediol, 2,3-pentanediol, 1,5-pentanediol, etc. can be substituted for the methylglycol and glycerol components in the procedures of the above examples with similar resulting advantage.

30 The invention has been described in detail with particular reference to preferred embodiments thereof, but, it will be understood that variations and modifications can be effected within the spirit and scope of the invention described hereinabove and in the appended claims.

We claim:

1. A process for spectrally sensitizing photographic silver halide which comprises: dispersing a substantially water-insoluble photographic spectral sensitizing dye in a water-soluble organic liquid which is a non-solvent for said dye; and, incorporating said dispersion into a liquid photographic silver halide emulsion, said organic liquid having the following formula:



45 50 wherein R represents a member selected from the group consisting of a hydrogen atom and an alkyl group containing from 1 to 4 carbon atoms; R<sub>1</sub> represents a member selected from the group consisting of a hydrogen atom and a methyl group; R<sub>2</sub> represents a member selected from the group consisting of a hydrogen atom, an alkyl group containing from 1 to 3 carbon atoms, a hydroxy-alkyl group of from 1 to 3 carbon atoms and an acetoxyethyl group; and, R<sub>3</sub> represents a divalent alkylene group containing from 1 to 4 carbon atoms, the sum of the carbon atoms in said R<sub>1</sub>, R<sub>2</sub> and R<sub>3</sub> being from 1 to 4.

55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 88

3. The process for spectrally sensitizing silver halide in accordance with claim 1 wherein the dispersion of dye in organic liquid is mixed with an aqueous solution of a hydrophilic colloid to form a homogenous mixture and said mixture is incorporated into the light-sensitive silver halide emulsion.

4. The process for spectrally sensitizing silver halide in accordance with claim 3 wherein said aqueous mixture of dye, organic liquid and hydrophilic colloid is dried prior to incorporation into said light-sensitive silver halide emulsion.

5. A process for spectrally sensitizing photographic silver halide which comprises: dispersing in methylglycol a photographic spectral sensitizing dye selected from the group consisting of

1'-ethyl-2-methylthia-4'-cyanine salt;  
3,3'-diethyl-9-methylselenacarbocyanine salt;  
1,1'-diethyl-2,2'-cyanine salt;  
3-ethyl-5-[(3-ethyl-2(3H)-benzothiazolylidene)isopropylidene]-2-thio-2,4-oxazolidinedione;  
9-ethyl-3,3'-di(β-methoxyethyl)-5,5'-diphenyloxacarbocyanine salt;  
anhydro-5',6,6'-tetrachloro-1,1'-diethyl-3,3'-di(3-sulfobutyl)-benzimidazolocarbocyanine hydroxide;  
5-[(3-ethyl-2(3H)-naphtho[2,1]oxazolylidene)ethylene]-3-n-heptyl-1-phenyl-2-thiohydantoin;  
5-(3-ethyl-2(3H)-benzoxazolylidene)-3-phenylrhodanine;  
anhydro-5,5'-dichloro-3,9-diethyl-3'-(3-sulfobutyl)thiocabocyanine hydroxide;  
5-[di(3-ethyl-2(1H)-naphtho[1,2]thiazolylidene)isopropylene]-1,3-di(β-methoxyethyl) barbituric acid; and  
3-ethyl-5-[1-(4-sulfobutyl)-4(1H)-pyridylidene]rhodanine, sodium salt;

and incorporating said dispersion into an aqueous gelatin photographic silver halide emulsion to spectrally sensitize the silver halide.

6. The process in accordance with claim 5 wherein the dispersion of dye in methylglycol is mixed with an aqueous solution of gelatin to form a homogeneous mixture, and said mixture is incorporated into said photographic silver halide emulsion.

7. The process for spectrally sensitizing silver halide in accordance with claim 5 wherein said mixture is dried prior to incorporation into the photographic silver halide emulsion.

8. A process for spectrally sensitizing photographic silver halide which comprises: dispersing in glycerol a photographic spectral sensitizing dye selected from the group consisting of

1'-ethyl-2-methylthia-4'-cyanine salt;  
3,3'-diethyl-9-methylselenacarbocyanine salt;  
1,1'-diethyl-2,2'-cyanine salt;  
3-ethyl-5-[(3-ethyl-2(3H)-benzothiazolylidene)isopropylidene]-2-thio-2,4-oxazolidinedione;  
9-ethyl-3,3'-di(β-methoxyethyl)-5,5'-diphenyloxacarbocyanine salt;  
anhydro-5',6,6'-tetrachloro-1,1'-diethyl-3,3'-di(3-sulfobutyl)-benzimidazolocarbocyanine hydroxide;  
5-[(3-ethyl-2(3H)-naphtho[2,1]oxazolylidene)ethylene]-3-n-heptyl-1-phenyl-2-thiohydantoin;  
5-(3-ethyl-2(3H)-benzoxazolylidene)-3-phenylrhodanine;  
anhydro-5,5'-dichloro-3,9-diethyl-3'-(3-sulfobutyl)thiocabocyanine hydroxide;  
5-[di(3-ethyl-2(1H)-naphtho[1,2]thiazolylidene)isopropylene]-1,3-di(β-methoxyethyl) barbituric acid; and  
3-ethyl-5-[1-(4-sulfobutyl)-4(1H)-pyridylidene]rhodanine, sodium salt;

and, incorporating said dispersion into an aqueous gelatin photographic silver halide emulsion.

9. A process for spectrally sensitizing photographic silver halide which comprises: dispersing a substantially

water-insoluble photographic spectral sensitizing dye in a water-soluble organic liquid mixture without dissolving the dye, said organic liquid mixture comprising about 80 to 95 parts by weight of an organic liquid selected from the group consisting of an alcohol having from 1 to 4 carbon atoms, acetone and dimethylformamide, and, about 20 to 5 parts by weight of an organic liquid having the following formula:



wherein R represents a member selected from the group consisting of a hydrogen atom and an alkyl group containing from 1 to 4 carbon atoms; R<sub>1</sub> represents a member selected from the group consisting of a hydrogen atom and a methyl group; R<sub>2</sub> represents a member selected from the group consisting of a hydrogen atom, an alkyl group containing from 1 to 3 carbon atoms, a hydroxyalkyl group of from 1 to 3 carbon atoms and an acetoxy-methyl group; and, R<sub>3</sub> represents a divalent alkylene group containing from 1 to 4 carbon atoms, the sum of the carbon atoms in said R<sub>1</sub>, R<sub>2</sub> and R<sub>3</sub> being from 1 to 4; and, incorporating said dispersion into a liquid photographic silver halide emulsion to spectrally sensitize the silver halide.

10. A process as defined in claim 9 wherein said organic liquid mixture comprises about 80 to 95 parts by weight methanol and about 20 to 5 parts by weight glycerol.

11. A process for spectrally sensitizing silver halide which comprises: dispersing, in about 5 cc. of an organic liquid mixture comprising 9 parts by weight methanol and 1 part by weight glycerol, about .5 gram of 3-ethyl-5-[(3-ethyl-2(3H)-benzothiazolylidene)isopropylidene]-2-thio-2,4-oxazolidinedione.

12. A mixture comprising a hydrophilic colloid and a dispersion of a photographic spectral sensitizing dye in a water-soluble organic liquid in which the dye is insoluble, said organic liquid having the following formula:



wherein R represents a member selected from the group consisting of a hydrogen atom and an alkyl group containing from 1 to 4 carbon atoms; R<sub>1</sub> represents a member selected from the group consisting of a hydrogen atom and a methyl group; R<sub>2</sub> represents a member selected from the group consisting of a hydrogen atom, an alkyl group containing from 1 to 3 carbon atoms, a hydroxyalkyl group of from 1 to 3 carbon atoms and an acetoxy-methyl group; and R<sub>3</sub> represents a divalent alkylene group containing from 1 to 4 carbon atoms, the sum of the carbon atoms in said R<sub>1</sub>, R<sub>2</sub> and R<sub>3</sub> being from 1 to 4.

13. A mixture comprising a hydrophilic colloid and a dispersion as defined in claim 12 wherein said organic liquid is selected from the group consisting of glycerol, monoacetin, ethylene glycol, methylglycol, ethyl glycol ether, propyl glycol ether, butyl glycol ether, 1,3-propylene glycol, 1,3-butylene glycol, 1,4-butylene glycol, 2,3-butylene glycol, isobutylene glycol, 2-methyl-2,3-butanediol, 3-methyl-1,3-butanediol, 1,2-pentanediol, 1,4-pentanediol, 2,3-pentanediol and 1,5-pentanediol.

#### References Cited

#### UNITED STATES PATENTS

3,469,987 9/1969 Owens et al. 96—132

70 J. TRAVIS BROWN, Primary Examiner

U.S. Cl. X.R.

96—132, 134, 137, 139, 140